

## UNITED STATES PATENT OFFICE

2,225,589

## PROCESS FOR THE REFINING OF TEXTILES

Hans Haussmann, Mannheim, and Oswald Meissner, Walter Pinkernelle, and Helmut Zinke, Uerdingen, Germany, assignors to I. G. Farbenindustrie Aktiengesellschaft, Frankfort-on-the-Main, Germany

No Drawing. Application April 13, 1937, Serial No. 136,636. In Germany April 18, 1936

13 Claims. (Cl. 8—120)

This invention relates to the refining of textiles.

It is already known to refine natural or artificial textiles, such as for example, cotton, wool, fibres of regenerated cellulose or cellulose esters or cellulose ethers by incorporating into the textiles by chemical means the radicles of the water repelling fatty acids originally contained in the natural fibres, but which have been eliminated 10 during the preliminary treatment thereof.

In accordance with the present invention it is now no longer necessary to be restricted for this purpose to the incorporation of fatty acid radicles and moreover, the properties to be imparted 15 to the textiles can likewise be attained by the incorporation of the radicles of dibasic carboxylic acids forming inner anhydrides and containing saturated or unsaturated open or cyclic carbon chains of at least 7 carbon atoms and especially 20 of at least 9 carbon atoms.

Among the acid radicles of the kind specified are particularly adapted for use in the present invention the radicles of succinic acids substituted in at least one methylene group by a 25 hydrocarbon radicle of at least 7 carbon atoms for example by at least one saturated alkyl radicle of at least 7 carbon atoms and especially 9 carbon atoms, such as heptyl succinic acid, octyl succinic acid and especially isononyl succinic 30 acid, isododecyl succinic acid and pentadecyl succinic acid, the anhydrides of these acids being obtainable for example in accordance with the co-pending application Ser. No. 733,126, filed June 29, 1934, by condensing saturated hydro- 35 carbons, such as heptane, octane and especially isononane, isododecane and pentadecane with maleic anhydride. Furthermore the radicles of succinic acids substituted in at least one methylene group by at least one unsaturated 40 alkyl radicle of at least 7 carbon atoms and especially 9 carbon atoms, such as isononetyl succinic acid, isododecetyl succinic acid, pentadecetyl succinic acid and octadecetyl succinic acid are suitable for the purpose of this invention, the 45 anhydrides of these acids being obtainable for example by condensing the corresponding olefines, such as isononylene, isododecylene, pentadecylene and octadecylene with maleic anhydride (compare French Patent No. 801,919). 50 Finally are to be mentioned the radicles of succinic acids substituted in at least one methylene group by at least one aralkyl radicle, such as  $\gamma$ -methyl- $\gamma$ -phenylpyrotartaric acid and  $\gamma$ -phenyl- $\gamma$ -dimethylpyrotartaric acid, anhydrides of succinic acids of this type being obtainable for ex-

ample by the process of the co-pending application Ser. No. 733,126 by condensing aliphatic hydrocarbons substituted by an aromatic radicle, such as toluene, ethyl benzene, diethyl benzene, propyl benzene and isopropyl benzene, diisopropyl benzene, triisopropyl benzene, teraphenylbenzene etc. with maleic acid anhydride. 5

The chemical incorporation of the acid radicles into the textiles proceeds in the manner known per se, that is to say, the fibres are subjected to esterification by means of the said acid radicles under mild reaction conditions. For attaining esterification it suffices generally to treat the textiles, such as for example artificial fibres of regenerated cellulose or cotton materials at a 15 temperature over about 30° C. and especially from about 60 to about 70° C. with a solution of an anhydride of the type of acid indicated in a suitable solvent which is inert under the reaction conditions such as carbon tetrachloride, chloroform, acetone, esters of organic acids, for example ethyl acetate, butyl acetate etc. 20

The degree of the hydrophobe action can be increased by subjecting the fibres treated in the manner described before after allowing the excess solution to drain off to an after-heating over about 100° C. and especially from about 110 to about 130° C. 25

Furthermore it has been found that by the esterification of the fibres at a temperature up to about 70° C. in the manner described above only one carboxyl group of the dibasic carboxylic acids is esterified with the textile fibre while the other carboxyl group remains free and that even at the after-treatment at a temperature up to about 35 130° C. still part of the carboxyl acid groups remain in a free condition. It has now been found that the hydrophobe qualities of the textile materials treated in the manner described before can be improved considerably by subjecting them 40 to an after-treatment with a salt forming agent whereby the free carboxyl groups are combined with a base which is so selected that the capacity for taking up water is still further reduced. 45

The salt formation can be carried out in the manner known per se, as for example, by the interaction of the acid groups with bases, such as especially bases of polyvalent metals, for example calcium hydroxide, zinc oxide, aluminium hydroxide, cerium oxide or with metal salts and especially salts of polyvalent metals of weak acids, such as calcium bicarbonate, aluminium formate, zinc acetate, furthermore for example in such a manner that there is first formed with the carboxyl group a water-sensitive salt, for ex- 50 55

- ample an alkali salt, such as sodium, potassium or ammonium salt by the interaction of a corresponding base such as a hydroxide of the alkali metals mentioned before or a weak acid salt of 5 these alkali metals such as a carbonate and the water-sensitive salt formed is then converted by double decomposition with a corresponding different salt especially of a polyvalent metal, such as calcium chloride, zinc sulfate, aluminium 10 sulfate or lead chloride into a water-insensitive salt.
- Particularly good results are produced by salt formation with polyvalent metals, such as calcium, zinc, aluminium, cerium and lead.
- 15 The following examples will illustrate the invention without being restricted thereto:

*Example 1*

- Dyed cotton material is treated for a short time 20 at a temperature of 60° C. with a solution consisting of 5 gms. of the anhydride of dodeceny succinic acid per litre of carbon tetrachloride and subjected for an hour at a temperature of 120° C. after vaporising the solvent. In this manner 25 a very good waterproof effect is attained, which even withstands boiling with soap and sodium carbonate for half an hour.

*Example 2*

- 30 Cotton materials which are frequently washed, for example, materials for wind jackets, are dipped for a short time in a solution of 5 gms. of the anhydride of isononetyl succinic acid per litre of benzine and squeezed out. After removing 35 the solvent the goods are hung in a drying chamber at 120° C. for an hour. In this manner a fabric is obtained with very good water repellent properties which are maintained after repeated washing by boiling.

*Example 3*

- Cotton fabric is treated for 15 minutes at 65° C. with a 0.6% solution of isopentadecenyl succinic acid anhydride in carbon tetrachloride. The 45 material is then beaten until air dry and rinsed with well water comprising 0.04% calcium bicarbonate per litre for 5 minutes at 80° C., dried over night and on the next day again rinsed for 5 minutes at 80° C. with the same well water. 50 By this means the calcium bicarbonate present in the well water causes the formation of the calcium salt with the free carboxyl groups in the fabric.

After drying, the fabric, when tested by the 55 standard method, shows a water pressure number of 105 mm., whereas the water pressure number of the untreated fabric is practically zero.

*Example 4*

- 60 In the same manner as in Example 1 cotton fabric is treated with a 0.6% carbon tetrachloride solution of a substituted succinic acid anhydride obtained by condensation of triisopropyl benzene with maleic acid anhydride. The material is 65 rinsed with well water as in Example 1 and dried.

*Example 5*

- An artificial silk fabric consisting of regenerated cellulose is treated with a 0.6% carbon 70 tetrachloride solution of 'n'-octadecenyl-succinic acid anhydride for about 15 minutes at 65° C. and after beating air dry, treated for 5 minutes with a dilute aqueous 3% sodium carbonate solution at 80° C. The material is then introduced for 5 minutes into an aqueous zinc chloride so-

lution heated to 80° C. After squeezing out and drying there is obtained on sprinkling the material with water a moisture absorption of 36%, whereas the untreated fabric tested in a similar manner takes up 100% of moisture.

*Example 6*

The fabric is treated with 'n'-octadecenyl succinic acid anhydride as in Example 5. After rinsing in dilute sodium carbonate solution, instead of the treatment in a zinc chloride bath a treatment in an alum bath is carried out.

We claim:

1. Process which comprises esterifying material selected from the group consisting of cotton and artificial regenerated cellulose fibres with an inner anhydride of a succinic acid substituted in at least one methylene group by at least one hydrocarbon radicle of at least 9 carbon atoms, and subjecting the material treated in this manner to an after-treatment with an agent forming a water-insoluble salt with the free carboxylic acid groups on the fibre.

2. Process which comprises esterifying material selected from the group consisting of cotton and artificial regenerated cellulose fibres with an inner anhydride of a succinic acid substituted in at least one methylene group by at least one hydrocarbon radicle of at least 9 carbon atoms, and subjecting the material treated in this manner to an after-treatment with an aqueous solution of a weak acid salt of a polyvalent metal.

3. Process which comprises esterifying material selected from the group consisting of cotton and artificial regenerated cellulose fibres with an inner anhydride of a succinic acid substituted in at least one methylene group by at least one hydrocarbon radicle of at least 9 carbon atoms, and subjecting the material treated in this manner to an after-treatment with an aqueous solution of calcium bicarbonate.

4. Process which comprises esterifying material selected from the group consisting of cotton and artificial regenerated cellulose fibres with an inner anhydride of a succinic acid substituted in at least one methylene group by at least one hydrocarbon radicle of at least 9 carbon atoms, and subjecting the material treated in this manner to an after-treatment with an agent forming a water-sensitive salt with the free carboxylic acid groups on the fibre, and then converting this salt with a corresponding different salt into a water-insoluble salt.

5. Process which comprises esterifying material selected from the group consisting of cotton and artificial regenerated cellulose fibres with an inner anhydride of a succinic acid substituted in at least one methylene group by at least one hydrocarbon radicle of at least 9 carbon atoms and subjecting the material treated in this manner to an after-treatment with an alkali carbonate solution, and then treating the alkali salt formed with a polyvalent metal salt solution.

6. Refined water-repellent textiles which contain the radicle of a dibasic carboxylic acid capable of forming an inner anhydride and having a carbon chain of at least 7 carbon atoms, one carboxylic acid group of which is in the form of a water-insoluble salt radicle.

7. Material selected from the group consisting of water-repellent cotton and water-repellent artificial regenerated cellulose fibres which contain a radicle of succinic acid substituted in at least one methylene group by at least one hydrocarbon radicle of at least 9 carbon atoms, one

- carboxylic group of that acid being in the form of a water-insoluble salt radicle.
8. Material selected from the group consisting of water-repellent cotton and water-repellent artificial regenerated cellulose fibres, which contain a radicle of succinic acid substituted in at least one methylene group by at least one hydrocarbon radicle of at least 9 carbon atoms, one carboxylic group of that acid being in the form of a calcium salt radicle.
9. A refined water-repellent cotton fabric containing the radicle of isopentadecenyl succinic acid, one carboxylic acid group of which is in the form of a calcium salt radicle.
10. A refined water-repellent regenerated cellulosic fabric, which contains the radicle of n-octadecenyl succinic acid, one carboxylic acid group of which is in the form of a zinc salt radicle.
11. The process which comprises chemically reacting cotton fabrics at 65° C. with a solution of isopentadecenyl succinic acid anhydride in carbon tetrachloride for a sufficient period of time and concentration of anhydride to render the fabrics water repellent, drying the fabric and then rinsing the same with water containing calcium bicarbonate to thereby increase the water repellency of the treated fabrics.
12. The process which comprises chemically reacting regenerated cellulose fabrics at a temperature of 65° C. with a solution of n-octadecenyl succinic acid anhydride in carbon tetrachloride, for a sufficient period of time and concentration of anhydride to render the fabrics water-repellent, drying the fabrics, then treating the fabrics with an aqueous sodium carbonate solution at a temperature of 80° C. and then with an aqueous zinc chloride solution at the same temperature, to thereby increase the water-repellency of the treated fabrics.
13. The process which comprises chemically reacting a textile with an inner anhydride of a di-basic carboxylic acid having a carbon chain of at least 7 carbon atoms at a concentration of anhydride, temperature and for a period of time sufficient to render the fabrics water-repellent, subjecting the textile treated in this manner to an aftertreatment with an agent forming a water-insoluble salt with the free carboxylic acid groups on the fiber to increase the water repellency of the fabrics.

HANS HAUSSMANN.  
OSWALD MEISSNER.  
WALTER PINKERNELLE.  
HELMUT ZINKE.

25